

## UNITED STATES PATENT OFFICE

2,224,448

## WEAR RESISTING ALLOY

Robert W. Schlumpf, Houston, Tex., assignor to  
 Hughes Tool Company, Houston, Tex., a corpora-  
 tion of Delaware

No Drawing. Application May 25, 1940,  
 Serial No. 337,249

4 Claims. (Cl. 75—126)

This invention relates to wear resisting me-  
 tallic alloys adapted for use as a hard facing  
 material or in the casting of small objects such  
 as nozzles for sand blasting devices or for well  
 5 drill nozzles, or similar articles.

It is an object to produce a hard alloy of  
 comparatively low melting point and adapted to  
 be fused in position at temperatures below the  
 fusing point of the objects to be hard faced.

10 It is also desired to provide a hard compound  
 which may be applied in position upon a device  
 by a casting operation in a furnace.

15 The general object of the invention is to pro-  
 vide a ferrous alloy which is of great hardness  
 and also which fuses at temperatures below  
 the melting point of ordinary steel, preferably  
 within the range of 2000° to 2300° F.

20 In forming this alloy I employ with the iron,  
 a small proportion of ingredients such as car-  
 bon, manganese and silicon which are desirable  
 in producing a good quality of steel. To these  
 elements, I add from 3 1/2% to 6 1/2% each of  
 25 chromium, molybdenum, and tungsten. To ob-  
 tain a low fusing point, I also add a small pro-  
 portion from 1% to 2% of boron.

The proportions of the different elements may  
 be varied within limits and I find that good re-  
 sults are obtained within the proportions indi-  
 cated in the following table:

|               | Per cent            |
|---------------|---------------------|
| Carbon        | 1.00 to 3.50        |
| Manganese     | 0.50 to 2.00        |
| Silicon       | 0.50 to 2.00        |
| Chromium      | 3.50 to 6.50        |
| 35 Molybdenum | 3.50 to 6.50        |
| Tungsten      | 3.50 to 6.50        |
| Boron         | 1.00 to 2.00        |
| Iron          | Balance to make 100 |

40 This compound fuses at comparatively low  
 temperatures ranging from 2000° to 2300° F. and  
 may be readily cast in position upon an object  
 such as a bearing, a cutter, or the like.

The object to be hard faced may be placed in a  
 mold, pieces of my alloy are then placed in the  
 mold and the object and mold placed in a fur-

nace and heated to a temperature above 2000° F.  
 to melt the alloy so that it will run down about  
 the object to be hard faced. This operation is  
 preferably performed in a non-oxidizing atmos-  
 phere. The mold is then cooled and the opera-  
 5 tion is completed except for such subsequent  
 machining as may be desired.

While the method described is preferable it  
 is to be understood that the alloy may be ap-  
 plied by other methods well known in the art 10  
 and the invention is not limited to the method  
 of application described.

What I claim as new is:

1. A hard alloy melting between 2000° and  
 2300° F. comprising elements fused together in 15  
 approximately the following proportions:

|            | Per cent            |
|------------|---------------------|
| Carbon     | 1.00 to 3.50        |
| Manganese  | 0.50 to 2.00        |
| Silicon    | 0.50 to 2.00        |
| Molybdenum | 3.50 to 6.50        |
| Tungsten   | 3.50 to 6.50        |
| Chromium   | 3.50 to 6.50        |
| Boron      | 1.00 to 2.00        |
| Iron       | Balance to make 100 |

2. A hard metal alloy melting below the fusing  
 point of steel comprising from 0.50% to 2.00%  
 30 each of silicon and manganese; approximately  
 2% each of carbon and boron, and approximately  
 5% of each of molybdenum, tungsten and chro-  
 mium and iron to make up 100% in all.

3. A hard metal alloy of comparatively low  
 melting point, consisting of not in excess of  
 3.50% carbon; manganese and silicon approxi-  
 35 mately 1% of each; molybdenum, tungsten and  
 chromium approximately 5% each; boron from  
 1 to 2%, and about 80% iron.

4. A hard metal alloy consisting of about 2%  
 of carbon; approximately 5% each of molyb-  
 denum, tungsten and chromium; 1% to 2% of  
 40 boron, about 1% each of manganese and silicon  
 and about 80% iron.

ROBERT W. SCHLUMPF.